

## UNITED STATES PATENT OFFICE

2,643,175

TREATMENT WITH ALCOHOLIC SOLUTION  
TO COMPLETE COUPLING OF AZO DYES  
IN CELLULOSE ACETATE TEXTILE MA-  
TERIALVictor S. Salvin, Irvington, N. J., assignor to Cela-  
nese Corporation of America, New York, N. Y.,  
a corporation of DelawareNo Drawing. Application December 5, 1950,  
Serial No. 199,363

1 Claim. (Cl. 8—48)

**1** This invention relates to the dyeing of textile materials and relates more particularly to an improved process for the dyeing by azoic methods of textile materials made of or containing yarns and filaments having a basis of cellulose acetate or other organic derivative of cellulose.

An object of this invention is the provision of an improved process for the dyeing of cellulose acetate or other organic derivative of cellulose textile materials with azo dyestuffs, and particularly with naphthol base azo dyestuffs.

Another object of this invention is the provision of an improved azoic dyeing process for the dyeing of cellulose acetate or other organic derivative of cellulose textile materials whereby true, deep shades of blue, which may be duplicated, may be obtained employing naphthol base developed azo dyestuffs to dye said textile materials.

A further object of this invention is the dyeing of cellulose acetate or other organic derivative of cellulose textile materials with developed naphthol base azo dyestuffs whereby colorations in true blue shades and of excellent resistance to light and crocking may be obtained.

Other objects of this invention will appear from the following detailed description.

The dyeing of textile materials with developed naphthol base azo dyestuffs has long been employed as a method for the dyeing of cellulosic textile materials such as cotton, or regenerated cellulose prepared by the viscose process. By this process, a range of heavy shades can be obtained and the resultant dyed cellulose textile materials exhibit outstanding fastness to washing as well as good resistance to light and to crocking. The application of this method of dyeing to textile materials having a basis of cellulose acetate or other organic derivative of cellulose has not, however, been as satisfactory as it is in the case of cotton or regenerated cellulose textile materials. This is particularly true in the case of dyeings in heavier shades which employ components normally yielding blue colorations on cotton or regenerated cellulose materials. Peculiarly enough, azo components which yield desirable, heavy true blue shades on cotton or regenerated cellulose materials do not yield the equivalent shade on cellulose acetate or other organic derivative of cellulose textile materials even though the same dyeing and coupling technique is employed. Not only has it been found that the results obtained cannot be duplicated with given coupling components but it has also been observed that the blue colorations on

**2** cellulose acetate or other organic derivative of cellulose textile materials are not true blue shades and tend to appear as plum and purple shades. Furthermore, these dyeings do not exhibit particularly satisfactory wash fastness or light fastness and they are also quite prone to crocking.

I have now found that cellulose acetate or other organic derivative of cellulose textile materials may be dyed satisfactorily, and in true shades, with developed naphthol base azo dyestuffs by azo coupling operations utilizing suitable developers if certain modifications are made in the usual procedures heretofore employed. In accordance with my process, I have found that improved dyeings may be obtained on cellulose acetate or other organic derivative of cellulose textile materials with naphthol base azo dyestuffs if a condition of low acidity exists during diazotization and, more importantly, if the proper degree of penetration and as complete coupling as possible is achieved during the development of the dyeings in said dyeing operations.

I have found that the condition of low acidity during diazotization has the highly advantageous effect of reducing the extent to which nitroso naphthols form during the diazotization reaction. The formation of nitroso naphthols is quite undesirable during diazotization since these compounds tend to produce off-shades and, in addition, appear to be responsible for a lack of light fastness in the dyed textile material. The low acidity during diazotization is readily achieved by employing an organic acid of low acidity such as, for example, acetic acid or formic acid in lieu of the excess of mineral acid, such as hydrochloric acid, normally employed during diazotization. Preferably, I employ acetic acid to attain the desired degree of acidity and in amounts of 0.3 to 0.5% by weight on the weight of the aqueous diazotization bath employed. The diazotization of the amines employed as coupling components for coupling with the naphthol base is otherwise carried out in the usual way employing sodium nitrite to convert the amine to the diazo compound. The use of temperatures of 20 to 40° C. over a period of 20 to 40 minutes is satisfactory in order to effect complete diazotization of the amine. Usually, from about 0.2 to 0.3% by weight of sodium nitrite is employed in the diazotization bath.

To achieve an increased degree of penetration during development, various expedients may be employed. Thus, for example, increased pene-

tration may be attained by increasing the temperature of development. Particularly advantageous results are attained when development is effected at temperatures of 75 to 90° C., or higher, in an alkaline aqueous soap solution. In addition to an increase in the degree of penetration, an appreciable increase in the speed of penetration is also attained. The combined effect of these desirable changes is a noticeable improvement in shade, particularly in the case of blue dyeings. Higher temperature also favors a more complete reaction so that any incompletely reacted nitroso naphthols present are held to a minimum. Increased penetration with the production of desirable true shades, and particularly blue shades, may also be achieved by merely increasing the time of development in the aqueous soap solution employed so that not only will the coupling reaction be more complete but the increased time permitted will allow the desired increased degree of penetration to be achieved to produce the true blue shades desired. Preferably, the aqueous alkaline developing bath is maintained at a pH of 7.5 to 9.0.

Highly advantageous results may also be attained by adding agents having a swelling or solvent action on the cellulose acetate or other organic derivative of cellulose textile material being dyed to the aqueous alkaline soap solution in which development is carried out. Preferably, however, I obtain the increased degree of penetration desired after the development of the dyestuff on the textile material is completed in the aqueous alkaline bath, by passing the textile material carrying the developed dyestuff through a bath containing such a swelling agent. Examples of suitable swelling agents are ethyl alcohol, the monobutyl ether of diethylene glycol, diacetone alcohol, triethyl phosphate or the mono-butyl ether of ethylene glycol. In lieu of employing a treating bath containing the swelling agent, the textile material carrying the developed dyestuff may be exposed to vapors of a suitable volatile swelling agent, e. g. ethyl alcohol or methyl ethyl ketone. Particularly advantageous results are obtained by the latter method since only a very short exposure to said vapors is necessary to produce the desired penetration. Certain dispersing agents also yield valuable results and in this connection there may be mentioned the nonionic dispersing agents obtained by the condensation of diethanolamine with long chain fatty acids, such as oleic, lauric, stearic and ricinoleic acid.

Thus, various means may be employed to achieve an increased penetrating action either during development, or subsequently, and to obtain as complete a reaction as possible.

I have also found that thorough scouring of the dyed textile material after development has been completed employing an alkaline scouring bath at a temperature of 85 to 90° C. is highly advantageous. Thorough scouring acts to remove whatever loose particles of nitroso naphthols there may be present as well as any other loose dyestuff particles. The removal of these loose materials by thorough scouring has been found to give dyeings of noticeably improved light fastness. The high temperature employed for said scouring step also acts, in addition, to ensure complete coupling of any incompletely coupled components still present after the development, and after any one of the above after-treatments, whereby the degree of penetration is increased.

As in the usual process for the application of naphthol base azo dyestuffs, the coupling components may be applied to the textile material in various ways. One of the most convenient methods of applying the coupling components is by co-dyeing or simultaneously applying both the amine and the naphthol base to the fabric or other textile material and then entering the fabric into a diazotizing bath where diazotization and coupling takes place. Alternatively, the textile material may be prenaphtholated by incorporating the naphthol base which is employed in the yarns comprising the fabric during spinning operations. The fabric may also be prenaphtholated by being padded with an aqueous dispersion of the naphthol base and then dried. In order to carry out the coupling reaction, the naphtholated textile material may then be immersed in a bath containing the diazotized amine with which the naphthol base is to be coupled. The pre-naphtholated textile material may also be dyed with a dispersion of the amine coupling component and the textile material thus obtained passed into a bath in which diazotization of the amine takes place. The development of the dyeing, after diazotization, may then be carried out in any one of the several ways I have described whereby improved penetration is attained and with minimum formation of nitroso naphthols.

In order further to illustrate my invention, but without being limited thereto, the following examples are given:

*Example I*

35 A fabric woven of cellulose acetate yarn of an acetyl value of 54.9, calculated as acetic acid, is co-dyed with a dyebath in which the dyestuffs present are a mixture of 4-benzoyl-amino-2,5-diethoxy aniline and of the anilide of beta-oxy naphthoic acid in such proportion that 2% of the former and 2% of the latter is placed upon the fabric. The fabric is then diazotized at 20° C. for 30 minutes in a diazotizing bath containing 2 grams per liter of sodium nitrite and 5 grams per liter of acetic acid. The diazotized fabric is then rinsed and placed in a developing bath consisting of a soap solution containing one gram per liter of soap and buffered to a pH of 9. The fabric is maintained in said bath for 1 hour with the bath at a temperature of 85 to 90° C. The fabric is dyed a violet-blue shade having a 20 hour light fastness resistance as measured in accordance with the standard A. A. T. C. C. test. Employing a developing bath of the same composition and at a temperature of 65 to 70° C. for 1½ hours gives a purple blue shade with only a 10-hour light fastness resistance.

*Example II*

60 A cellulose acetate fabric is co-dyed and diazotized as described in Example I and is then entered into a developing bath, buffered to a pH of 9, and containing 0.2% by weight of soap and 2% by weight of the mono-butyl ether of diethylene glycol. The fabric is developed for 1 hour with the bath at a temperature of 75 to 80° C. The cellulose acetate fabric is dyed a royal blue shade having a 40 hour light fastness resistance.

*Example III*

A cellulose acetate fabric is dyed and diazotized as described in Example I and is then placed in an aqueous developing bath, buffered to a pH of 9 and containing 0.2% by weight of soap. The

fabric is maintained in the soap solution for  $\frac{1}{2}$  hour with the solution at a temperature of 65° C. The fabric is then removed and placed in a 50% by weight aqueous solution of ethyl alcohol at 25° C. for 1 minute. The developed fabric is then scoured and dried. The cellulose acetate fabric is dyed a true neutral blue shade exhibiting a light fastness resistance of 40 hours.

*Example IV*

A cellulose acetate fabric is dyed and diazotized as described in Example I and is then placed in a developing bath consisting of an aqueous 50% by weight solution of ethyl alcohol. The fabric is maintained in said solution at 25° C. for 3 minutes and is then removed and scoured. The fabric is found to be dyed in a true neutral blue shade having a light fastness resistance of 40 hours.

*Example V*

A cellulose acetate fabric is dyed and diazotized as described in Example I and is then exposed for 1 minute to vapors of ethyl alcohol at 80° C. The fabric is then scoured and dried and is found to be dyed a true neutral blue shade having a light fastness resistance of 40 hours.

While my invention has been more particularly described in connection with the use of an anilide of beta-oxy naphthoic acid known as Naphthol AS, equally advantageous results are obtained employing as the naphthol base, the ortho aniside of beta-oxy naphthoic acid (Naphthol AS/OL), the toluidine of beta-oxy naphthoic acid (Naphthol AS/D) and the ortho toluidide of hydroxy carbazol (Naphthol AS/LB) as well as other naphthol bases commercially employed for the production of naphthol base azo dyestuffs. As amino coupling components which may be employed in the production of improved dyeings in accordance with my novel process there may be mentioned 2-methoxy-4-nitro-aniline, ortho - nitro - aniline, ortho-amino-azo-toluene, paranitro-aniline and toluidine. It is to be understood, of course, that not all combinations of naphthol base and amino coupling components yield blue shades. However, my novel process is highly advantageous for increasing the fastness

of all of said naphthol base azo dyestuffs and, in the case of these combinations yielding blue dyeings, my novel process is highly advantageous for the production of true blue shades of increased resistance to light.

It is to be understood that the foregoing detailed description is given merely by way of illustration and that many variations may be made therein without departing from the spirit of my invention.

Having described my invention, what I desire to secure by Letters Patent is:

In a process for dyeing cellulose acetate textile materials with naphthol base azo dyestuffs, the steps which comprise applying a mixture of the naphthol base azo dyestuff components to a cellulose acetate textile material, effecting diazotization of said naphthol base azo dyestuff components on said textile material in a diazotizing bath containing acetic acid in amounts of 0.3 to 0.5% on the weight of the diazotizing bath, subjecting said cellulose acetate textile material carrying the azo dyestuff thereon to the action of a developing bath for said azo dyestuff and, after the development of said naphthol base azo dyestuff is completed, to the action of a bath containing 20 to 30% by weight of ethyl alcohol at a temperature of 20 to 30° C. for 1 to 3 minutes, whereby more complete coupling of said naphthol base azo dyestuff and increased penetration thereof in said cellulose acetate textile material are attained.

VICTOR S. SALVIN.

35 References Cited in the file of this patent  
UNITED STATES PATENTS

| Number    | Name        | Date          |
|-----------|-------------|---------------|
| 961,241   | Knoevenagel | June 14, 1910 |
| 2,048,786 | Ellis       | July 28, 1936 |
| 2,048,796 | Kirk        | July 28, 1936 |
| 2,090,669 | Dreyfus     | Aug. 24, 1937 |
| 2,218,628 | Sowter      | Oct. 22, 1940 |

FOREIGN PATENTS

| 45 Number | Country       | Date         |
|-----------|---------------|--------------|
| 470,333   | Great Britain | Aug. 6, 1937 |